

## UNITED STATES PATENT OFFICE

HAROLD J. ROSE, OF PENN TOWNSHIP, ALLEGHENY COUNTY, PENNSYLVANIA, AND  
WILLIAM H. HILL, OF ARLINGTON, NEW JERSEY, ASSIGNORS TO THE KOPPERS  
COMPANY OF DELAWARE, A CORPORATION OF DELAWARE

## COMPOSITION OF MATTER AND PROCESSES OF PREPARING THE SAME

No Drawing.

Application filed September 16, 1929. Serial No. 393,124.

This invention relates to compositions of matter and processes of preparing the same, and more particularly to the manufacture of products containing coal.

5 In a copending application of W. H. Hill, Serial No. 393,115, filed Sept. 16, 1929, plastic and coagulated masses are described which are produced by the addition of low boiling organic liquids or so-called volatile solvents 10 to coal solutions. Coal plastics prepared in this way are adapted to dry out by evaporation of the volatile solvent, leaving the original coal solution.

In accordance with the present invention, 15 a coal product of a coagulated nature and with certain very desirable properties may be prepared by the addition of certain organic materials, other than volatile solvents, which materials may be termed coagulating 20 agents, since it has been observed that the addition of proper proportions of these materials to coal solutions tends to convert dissolved coal into a suspensoid.

A product may be prepared which may be 25 of a gel nature and which may assume a gelatinous or jelly state. A gel is a product of a coagulated or plastic nature and may be here defined as a colloidally dispersed structure consisting of a solid and a liquid phase 30 or also of two viscous liquid phases, and having shape and cohesion, and elastic properties, although it may be very rich in liquid.

There results a formation of minute particles of undissolved coal in the coal solvent. 35 A given mass of treated coal solution may contain some dissolved coal and particles of undissolved coal or it may contain little or no dissolved coal, in which case substantially all of the previously dissolved coal is 40 changed to a suspensoid.

When coagulating agents are added to coal solutions in the proper proportions, it has been found that a product of a coagulated nature may be formed having a higher softening point than that of the original coal solution, but retaining a remarkable degree of softness. In other words, while the softening point of the product is higher than that of the original coal solution, the product retains the low degree of hardness of the

original coal solution at low temperatures. Thus the temperature susceptibility factor is greatly decreased by the addition of a coagulating substance.

The degree of the effects produced, and described above, can be controlled, and it depends on the particular coagulating agent added, on the amount of such agent, on the temperature of the coal solution or of the coagulating agent when about to be mixed, on the temperature to which the resulting mixture is heated and on the speed with which the coagulating agent is added. The consistency of the final product depends largely upon the above factors.

The present invention makes it possible to produce coagulated coal solutions of higher softening points without increasing the coal content. For instance, a given coal solution may be found to possess exactly the desired properties with respect to hardness at low temperatures but too low a softening point. Formerly there was only one method of overcoming this, that is, by increasing the coal content of the solution. This generally results in the loss of certain properties inherent in solutions containing lesser amounts of dissolved coal. The present invention makes it possible to increase the softening point to the desired higher temperatures without decreasing the percentage of solvent and still retain the desirable properties of the untreated coal solution.

As set forth in the copending application Serial No. 97,467, filed Mar. 25, 1926 by Rose and Hill, coal may be dissolved in oils such as coal tar or water-gas tar and certain distillates therefrom. The coal and oil are brought together and heated at normal or only moderately elevated pressures and moderately elevated but non-decomposing temperatures of from about 200° C. to about 400° C. Substantially all of the coal dissolves, forming homogeneous solutions which remain stable at temperatures below the point of rapid volatilization or even below the dissolving temperatures. The coals most easily dissolved in such solvents are generally the coking coals. Substantially all of such coals are soluble, the insoluble por-

tions consisting of the mineral matter or ash and the mineral charcoal or fusain which may be present in limited amounts.

Preferably a high boiling coke-oven-tar oil is used as a solvent for coal. Other oils such as cracked petroleum oils, and especially the higher boiling distillates thereof may also be used.

A coal solution may be prepared by heating one part of coal, such as Pittsburgh seam coal, and about three parts of crude coke-oven tar, for instance, in a closed vessel heated directly to a temperature of about 300° C., or below the temperature at which substantial decomposition of the coal takes place. Water and undesirable light oils are allowed to escape before the vessel is closed. The resulting product containing coal which is chemically unchanged, is allowed to cool and is discharged into containers at a temperature lower than the lowest boiling temperature (about 200° C.) of compounds contained therein.

In addition to the solvents for coal mentioned above, sulphur treated oils and tars described in the copending application of Rose and Hill, Serial No. 354,694, filed April 12, 1929, may also be used.

In accordance with the present process, a coal solution is prepared by dissolving coal in any of the solvents mentioned above, and any desired proportions of coagulating materials or reagents may be added to the resulting coal solution with stirring or kneading. The exact percentage of coagulating materials to be added depends upon the nature of the coal solution and the coagulating material and also upon the properties desired in the final product. Preferably, and in most cases, from about 1% to about 5% of coagulating materials may be added to a coal solution.

The coagulating materials used are preferably compounds of, or substances containing compounds of, the aliphatic series, such as paraffin oil, paraffin wax, lubricating oil, petroleum still residue, natural or blown asphalts, linseed oils, etc. It is desirable to employ coagulating materials of such high boiling points that they do not evaporate materially after the coagulated product has been applied.

In the use of drying oils such as linseed oil, tung oil or so-called Chinese wood oil, and so forth, as coagulating materials, it is noted that a product prepared with such oils becomes covered by a dense tough impermeable film of oxidized drying oil which is very advantageous in that it effectively reduces evaporation of the oils used as solvents for coal or other alterations in the coagulated coal solutions and thus reduces ageing to a minimum.

As an alternative, a product of this invention may be prepared by mixing a coagulating

material with a solvent for coal, adding coal thereto and heating the resulting mixture.

Some examples of the manner in which the products of this invention may be prepared are as follows:

Example 1.—95 parts by weight of coal solution containing 15% by weight of coal are melted and into it are slowly introduced with vigorous stirring 5 parts by weight of linseed oil.

Example 2.—80 parts by weight of coke-oven tar, topped to 400° F., and 5 parts by weight of paraffin oil are mixed and heated for two hours with 15 parts by weight of bituminous coal in a rotating autoclave at 610° F. The product is ready for use after it has cooled down to less than about 400° F.

Various inorganic and organic materials may be added to such coal solution products. The added materials may be of a purely inert type, as for instance pigments and fibres, such as clay, sand, mineral wool, asbestos, cellulose fibre, etc.; or they may exert some chemical or physical action, as for instance sulphur or its compounds.

Coagulated masses produced in accordance with the present invention may be called non-evaporative coagulated coal solutions. They are usually thickened coal solutions of a solid, semi-solid, plastic or semi-plastic nature and may be applied as a cold plaster or paste in thick layers without danger of drying out while preparing and applying them, or they may be applied as hot liquids. However, they may vary in consistency from a liquid to a solid and may be readily applied with a trowel, a putty knife or similar instrument without the use of heat.

A composition having remarkable elastic qualities may be produced which is particularly useful in the preparation of expansion joints. Non-evaporative coal gels or coagulated coal solutions may also be used as patching compounds for roofs, etc., or they may be used for renewing brake surfaces or in building up wearing surfaces. These products have excellent protective qualities and may be used as a water-proofing agent, as for instance, on ships' decks and so forth.

We claim as our invention:

1. A process of preparing bituminous products, which process comprises heating coal and oil solvent for coal together to non-decomposing temperatures of the coal, namely about 200° C. to 400° C., to form a homogeneous fluid mass, maintaining the said mass in a fluid state, and mixing with the said mass a composition of aliphatic nature selected from a group consisting of vegetable oil, paraffin oil, paraffin wax, lubricating oil, petroleum still residue, and asphalt in sufficient amount to form a thickened mass upon addition thereof.

2. A process of preparing bituminous products, which process comprises heating coal

and oil solvent for coal together in the form of a homogeneous fluid mass at a temperature below the temperature at which chemical decomposition of the coal takes place and  
5 mixing with the said fluid mass a composition of aliphatic nature selected from a group consisting of vegetable oil, paraffin oil, paraffin wax, lubricating oil, petroleum still residue, and asphalt in sufficient amount to form  
10 a thickened mass upon addition thereof.

3. A bituminous product comprising coal and solvent for coal which have been heated together to non-decomposing temperatures of about 200° C. to 400° C., and a composition of aliphatic nature selected from a group consisting of vegetable oil, paraffin oil, paraffin wax, lubricating oil, petroleum still residue, and asphalt in sufficient amount to form a thickened mass upon addition thereof.

20 4. A bituminous product comprising previously dissolved coal uniformly distributed in a solvent for the coal, and linseed oil distributed in the solvent in sufficient amount to cause separating out of coal from solution and  
25 to form a thickened mass upon addition of the said linseed oil.

5. A process of preparing bituminous products, which process comprises heating coal and oil solvent for coal together to non-decomposing temperatures of the coal, namely about 200° C. to 400° C., to form a homogeneous fluid mass, and thickening the said fluid mass by adding a relatively high-boiling liquid aliphatic composition which when added will  
35 increase the consistency of the said fluid mass while distributing the said composition in the said fluid mass.

In testimony whereof, I have hereunto subscribed my name this 5th day of September,  
40 1929.

HAROLD J. ROSE.

In testimony whereof, I have hereunto subscribed my name this 9th day of September,  
45 1929.

WILLIAM H. HILL.

50

55

60

65